

Dec. 13, 1955

J. E. HICKOK ET AL

2,726,993

PROCESS FOR IMPROVING LIQUID FUELS BY TREATING  
WITH PROPANOL AND A METAL PASSIVATOR

Filed Nov. 15, 1951



FIG.-1



FIG.-2

John E. Hickok  
George S. Tobias  
Robert V.J. McGee Inventors

By W.O. Heilman Attorney

## 1

2,726,993

**PROCESS FOR IMPROVING LIQUID FUELS BY  
TREATING WITH PROPYANOOL AND A METAL  
PASSIVATOR**

John E. Hickok, New Providence Township, Union County, George S. Tobias, Plainfield, and Robert V. J. McGee, Union, N. J., assignors to Esso Research and Engineering Company, a corporation of Delaware

Application November 15, 1951, Serial No. 256,534

4 Claims. (Cl. 196—44)

The present invention is concerned with a process for producing liquid petroleum fuels of high quality. The invention is more particularly concerned with a process for manufacturing gasolines, heating oils and other distillate fuels of high quality. Such fuels are mixtures of hydrocarbons and are used in internal combustion engines, like those with Otto or with Diesel cycle, in turbo-jet engines in aviation, and in various burner systems for domestic or industrial heating.

In accordance with the present invention, these fuels are treated with an alcohol, either alone or in conjunction with a metal-passivator, in a manner to produce improved fuels, stable against the formation of sediment, sludge, gum or similar products of deterioration. A metal-passivator is a salt that has the property of protecting ferrous metals from corrosion.

It is well known in the art to make fuels from petroleum feed-stocks by various refining operations, including straight distillation from crude oil and thermal or catalytic cracking. It is also well known in the art to treat distillate fuels, such as gasoline or heating oil, by various processes in order to remove sediment or sediment-forming impurities and thus to improve the quality and stability of the products. Examples of treating processes are acid-treating, caustic-washing and doctor-sweetening. In certain instances, further improvement in quality and stability has been achieved by the use of addition agents, for example anti-oxidants and detergents in the fuels.

However, the conventional refining and treating processes, particularly when applied to fuels consisting wholly or in part of cracked distillates, are not always completely adequate to prevent the formation of sediment during storage and use of the fuels. As a result, such fuels may form deposits when used in an engine or may cause clogging of filters, screens, orifices or conduits associated with the burner systems in which they are used.

It has now been discovered that improved fuels, particularly gasoline, turbo-jet fuel, kerosene, heating oil and diesel fuel, may be obtained by treating distillates with an alcohol and a metal-passivating salt solution. The invention is preferably applied to distillates containing 10% or more of stocks derived from thermal or catalytic cracking operations, having a vapor pressure below 13 pounds per square inch at 100° F., and boiling below 750° F. at atmospheric pressure. Examples of such distillates are aviation gasoline with about 7 pounds vapor pressure and about 320° F. final boiling point, motor gasoline with about 8 to 12 pounds vapor pressure and about 420° F. final boiling point, turbo-jet fuel with about 2 lbs. vapor pressure and 550° F. final boiling point, diesel fuels falling within ASTM specification D-975-48T (grades No. 1-D to 4-D inclusive) and fuel oils falling within ASTM specification D-396-48T (grades No. 1 to 6).

As pointed out heretofore, the invention broadly is concerned with the production of high quality distillate products utilizing an alcohol alone or in conjunction with a solution of a metal-passivating salt. Various alcohols

## 2

may be used, as for example, primary aliphatic alcohols having from one to five carbon atoms in the molecule, secondary aliphatic alcohols having from 3 to 5 carbon atoms in the molecule, tertiary aliphatic alcohols having 5 to 4 to 5 carbon atoms in the molecule, cyclic alcohols like cyclo-hexanol, phenols like catechol, hetero-cyclic alcohols like furfuryl or tetrahydrofurfuryl alcohol, unsaturated alcohols like vinyl or allyl alcohol, di-hydroxy alcohols like ethylene glycol or propylene glycol or butane diol, and poly-hydroxy alcohols like glycerol, etc. The aliphatic alcohols having up to 5 carbon atoms in the molecule are preferred and isopropanol is particularly preferred.

The amount of alcohol used may vary appreciably, as for example in the range from about 0.5% to 20% by volume based upon the amount of oil being treated. The preferred amount is in the range of about 1% to 5% by volume. The treating temperature may range from 60° F. in open vessels to 450° F. in closed systems. In general the effectiveness of the treatment increases with increasing temperature. However, a particularly convenient range of operating temperatures is between 80° F. and 212° F.; while an operating temperature of from about 100° F. to a temperature at or slightly above the normal boiling point, 181° F., of isopropanol is particularly convenient for that reagent.

The metal-passivating salts are salts of sodium, potassium, ammonium or organic amines with certain inorganic or organic acids. Generally, the sodium salts are preferred for reasons of convenience, economy and effectiveness; but ammonium salts may be used for products in which the possibility of entraining ash-forming constituents is desirably to be avoided; and amine salts may be used advantageously when enhanced oil-solubility of the reagent is desirable. The acidic component of the salt is selected from the group, chromate, bichromate, phosphate, phosphite, nitrate, nitrite, borate and benzoate. Amine nitrates like morpholine nitrite or diisopropyl amine nitrite are desirable for being ashless and being capable of sublimation. Sodium benzoate also sublimes. 30 Sodium chromate or bichromate is convenient to be used in treating gasoline but is less desirable for treating diesel fuels. Sodium phosphate is particularly effective for imparting both antioxidant and rust-preventive effects. Sodium nitrite is the preferred reagent for use in conjunction with isopropanol in the treating of a wide variety 40 of fuels.

The process of the present invention may be more fully understood by reference to the drawings illustrating embodiments of the invention. Figure 1 illustrates an operation wherein a distillate is treated in a first stage 50 with an alcohol and the alcohol is removed in a second stage. Figure 2 illustrates an operation wherein a distillate is treated optionally with a metal salt, which may conveniently be in the form of an aqueous solution, in a first stage and is treated with an alcohol in a second stage and is separated from the alcohol in a third stage.

Referring specifically to Figure 1, a distillate, which for the purpose of illustration is taken to be a heating oil containing more than 10% of cracked gas oil, is introduced into a first treating zone 1 by means of line 2 and is treated with an alcohol, for example isopropanol, introduced through line 3. The treated distillate and the alcohol are removed from zone 1 by means of line 4 and introduced into a second treating zone 5 wherein the alcohol is removed from the treated distillate through line 8 either by a stripping distillation or by selective extraction with a solution of metal-passivating salt, for example sodium nitrite, which is introduced through line 7 if desired. The treated distillate is removed from zone 5 by means of line 6 and further refined or handled as desired.

Referring again to Figure 1, in an alternate operation,

the feed stock is a wide-cut distillate containing fractions of gasoline or turbo-jet fuel components as well as gas oil fractions, for example a catalytically cracked distillate boiling from about 100° F. to 650° F. The distillate is treated with an alcohol boiling below 400° F. in zone 1 and is fractionally distilled in zone 5 so as to withdraw a treated gas-oil as a residual fraction by means of line 6 and to recover a treated gasoline and/or turbo-jet fuel, containing at least a portion of the alcohol in unreacted condition, as an overhead fraction by means of line 8. A small amount of a preferably sublimable metal-passivator is introduced through line 7 if desired. The gas oil is thus stabilized against sediment formation and the overhead fraction is stabilized against formation of either gum from oxidation in hot weather or ice from moisture contamination in cold weather.

Referring specifically to Figure 2, a distillate feed stock as described for Figure 1 is introduced into a first treating zone 10 by means of line 11. In zone 10, according to one embodiment of the invention, the feed stock is treated with a solution of metal-passivating salt, like sodium nitrite, introduced by means of line 12 and withdrawn by means of line 13; but if, as hereinafter mentioned, a treatment with metal-passivating salt is selected as the alternative treatment in a third treating zone, the treatment in zone 10 can economically be omitted; and the process then becomes the same as in Figure 1. From zone 10 the distillate is passed through line 14 to a second treating zone 15 wherein the distillate is treated with an alcohol introduced by means of line 16. The mixture of treated distillate and alcohol is transferred from zone 15 by means of line 17 to a third treating zone 18 wherein the mixture is so treated as to remove the alcohol from the treated distillate fuel. The treated fuel is removed from zone 18 by means of line 19 and handled as desired.

One method of treating in zone 18 is to remove the alcohol by fractional distillation, which is particularly effective when there is a considerable difference in boiling points between the alcohol and the treated fuel. The preferred method of treating in zone 18, particularly when the treatment in zone 10 is omitted as heretofore mentioned, is to bring the fuel into intimate contact with an aqueous solution of a metal-passivating salt of sodium. For the purpose of illustration, it is assumed that the alcohol is removed by a solution of sodium nitrite introduced into zone 18 by means of line 20 and withdrawn as an aqueous alcoholic solution by means of line 21. It is to be understood that any number and arrangement of zones may be employed with respect to the process described. For instance, the operations of treating with alcohol and of separating from alcohol may, if desired, be carried out consecutively, or even continuously, in a single vessel, although the illustrations show the treating and the separating in separate zones for purposes of clarity. It is also to be understood that any suitable means for securing better mixing and contact likewise may be used.

The process of the present invention may be more fully understood by the following examples.

#### EXAMPLE I

A gasoline containing more than 50% cracked naphtha, having a vapor pressure of about 11 lbs. per sq. in. at 100° F., and showing about 60% distilled at 212° F. by ASTM test method D-86 and a final boiling point of about 380° F., was mixed with 5% of isopropanol and agitated at 80° F. in the presence of air. The gum content of the gasoline blend was determined initially and at various intervals of time during a test lasting 16 hours. The gum content was determined by the General Motors method, which is carried out in the manner described in ASTM method D-381-50 but at a temperature of about 375° F. The method is intended to measure "existent gum"; but, of course, some gum is inevitably formed by

polymerization and oxidation of unsaturated hydrocarbons while the test is in progress, so that a slight decrease in "General Motors gum" after the treatment with alcohol is indicative of a decrease in the potential gum-forming tendency of the gasoline being treated. The test results were as follows:

| Time Elapsed From Start of Test, Hrs. | Gum Content of Gasoline Blend, Mgs./100 ML. |
|---------------------------------------|---------------------------------------------|
| 0                                     | 4.0                                         |
| 24                                    | 5.4                                         |
| 1½                                    | 6.2                                         |
| 2½                                    | 4.6                                         |
| 6                                     | 4.8                                         |
| 8                                     | 3.8                                         |
| 8½                                    | 2.8                                         |
| 9½                                    | 2.6                                         |
| 14                                    | 1.8                                         |
| 16                                    | 1.8                                         |

Thus, it is apparent that if a petroleum oil boiling in the range of motor gasoline is treated with an alcohol at room temperature in the presence of air, an improvement in the gum content of the fuel is obtained after the treatment has progressed for a sufficient length of time. In the absence of alcohol, the effect of air would be to increase the gum content of the fuel according to well-known oxidation and polymerization phenomena.

#### EXAMPLE II

Four one-gallon samples of a gasoline having the characteristics described in Example I were subjected to comparative tests. Two of the samples were duplicate control samples. The other two were treated with 2% by volume of isopropanol and represented duplicate test samples. The four samples were stored in bright iron cans of five-gallon capacity and the cans were fitted with air-vents. The storage lasted 200 days and the samples were tested at intervals for gum content as described in Example I and for peroxide number by a method in which ferrous sulfate is oxidized to ferric sulfate and the amount of ferric sulfate formed is measured by titration with titanous chloride. The results of the tests are summarized as follows:

*Averages of duplicate tests of gasoline stored with and without 2% of isopropanol*

| Days Stored | Gum, mg./100 ml. |         | Peroxide No. gm. Equivalents of Oxygen/1,000 liters |         |
|-------------|------------------|---------|-----------------------------------------------------|---------|
|             | With             | Without | With                                                | Without |
| 0           | 5                | 4       | 1                                                   | 1       |
| 49          | 5                | 5       | 2                                                   | 3       |
| 109         | 6                | 7       | 3                                                   | 4       |
| 130         | 8                | 14      | 3                                                   | 6       |
| 172         | 11               | 41      | 5                                                   | 18      |
| 200         | No test          | No test | 5                                                   | 34      |

It is apparent from the tabulation above, that, even without agitation, the treatment of gasoline with alcohol at ambient temperatures in the presence of air is effective in retarding the formation of gum and of peroxides which are well-known in the art to be associated with the formation of gum in gasoline.

#### EXAMPLE III

A sample of gasoline having the same general characteristics as shown in Example I was tested for "Copper Dish Gum" by being evaporated from a dish of polished copper on a steam bath. The test is an approximate measure of potential gum-forming characteristics of gasoline; because the copper metal acts catalytically to promote gum formation during the evaporation of the sample

from the heated dish. For comparative purposes the test was repeated with various volume percentages of isopropanol in the gasoline. In another comparable series of tests, corresponding volume percentages of acetone were blended in the gasoline. The following results were obtained:

|                     | Copper Dish Gum, mgs./100 ml. |    |    |    |     |
|---------------------|-------------------------------|----|----|----|-----|
|                     | 0                             | 1  | 2  | 5  | 10  |
| Vol. Percent Added: |                               |    |    |    |     |
| Isopropanol         | 117                           | 62 | 60 | 81 | 100 |
| Acetone             | 117                           | 58 | 50 | 53 | 80  |

From the foregoing it is evident that for this gasoline under the conditions of the copper dish gum test there is an optimum percentage of reagent at about 2% by volume. In this test acetone is even more effective than isopropanol from which it can be formed by catalytic oxidation. It is possible that the effectiveness of the alcohol is due in part to its being oxidized; but the possibility is merely conjectural.

#### EXAMPLE IV

For illustrating the effect of treating with metal-passivators, a sample of heating oil was selected. It was a blend consisting of about 25% catalytically cracked gas oil, 45% thermally cracked gas oil and 30% virgin gas oil and it had the following typical characteristics:

|                                  |        |
|----------------------------------|--------|
| Gravity, degrees API             | 34.1   |
| Color (Tag Robinson Colorimeter) | 11 1/4 |
| Pensky-Marten flash-point, ° F.  | 158    |
| Percent sulfur content           | 0.6    |
| Aniline-point, ° F.              | 130    |
| ASTM distillation:               |        |
| Initial boiling point, ° F.      | 342    |
| 50% off at ° F.                  | 484    |
| Final boiling point, ° F.        | 628    |

Four portions of the above heating oil were treated separately, each with an equal volume of an aqueous solution of a metal-passivating sodium salt. The aqueous solutions were separated from the treated oil in each instance and the oil was tested for its tendency to form sludge in accelerated sediment-forming tests and also for the tendency for iron to become rusted when immersed in the water-saturated oil. The accelerated tests were run at 212° F. in air and in a closed container under oxygen pressure. Comparative results were as follows:

| Treating agent            | None  | 10% Sodium Phosphate | 1% Sodium Nitrite | 10% Sodium Nitrite | 10% Sodium Chromate |
|---------------------------|-------|----------------------|-------------------|--------------------|---------------------|
| Accelerated Sediment:     |       |                      |                   |                    |                     |
| mgs./100 ml., in air      | 4     | 1                    | 3                 | 2                  | 3                   |
| mgs./100 ml., in oxygen   | 32    | 30                   | 31                | 20                 | 11                  |
| Rusting tendency, 12 days | Heavy | Light                | Trace             | None               | Medium              |

The samples of treated oil showed improved stability against the formation of sediment even under very severely accelerated oxidation and improved anti-rusting characteristics.

#### EXAMPLE V

For illustrating the effect of treating with various alcohols and related materials, samples of the same heating oil as described in Example IV were treated with the reagents in various concentrations. The sediment initially removable from the oil by filtration was measured, as

well as the accelerated sediment subsequently formed by heating in air. Comparative results were as follows:

| Treating Agent      | Percent | Sediment, Mgs./100 ml. |                    |
|---------------------|---------|------------------------|--------------------|
|                     |         | Initially Filterable   | Accelerated in Air |
| None <sup>1</sup>   |         | 0.5                    | 4                  |
| Isopropanol         | 1.20    | 0.2                    | <1                 |
| Methanol            | 5.0     | 1.0                    | <1                 |
| Dipropylene glycol  | 2.0     | 0.3                    | <1                 |
| Tripropylene glycol | <1      | 0.4                    | <1                 |
| Acetone             | 2.0     | 0.3                    | 1                  |
| Paraformaldehyde    | <0.5    | 0.4                    | 2                  |
| Pyrogallol          | <0.02   | 0.4                    | 1                  |
| Catechol            | 0.02    | 0.3                    | 1                  |

<sup>1</sup> Rusting tendency, 12 days—Heavy.

All of the treating agents listed in the table above were effective to some degree in improving the stability of the heating oil. Pyrogallol and catechol have anti-oxidant properties, but the other reagents have not. Consequently, the results must be interpreted as indicating an effect distinct from the inhibition of oxidation.

#### EXAMPLE VI

For illustrating the effect of removing the volatile and water-soluble alcohols from the treated fuels, samples of the same heating oil as described in Example IV were treated with isopropanol, which was separated from them, after the treatment, in various ways. Comparative results were as follows:

| Heating Oil Treated with Isopropanol | Percent Added | Sediment, Mgs./100 ml. |                | Pensky-Marten Flash-Point, ° F. |
|--------------------------------------|---------------|------------------------|----------------|---------------------------------|
|                                      |               | Filterable             | Accel'd in Air |                                 |
| None                                 | 0.5           | 0.5                    | 4              | 158                             |
| do                                   | 0.5           | 0.2                    | <1             | 106                             |
| Water-washing                        | 0.5           | 0.1                    | 2              | 158                             |
| Distilled to 365° F.                 | 0.5           | 0.8                    | 1              | 176                             |
| None                                 | 5.0           | 0.3                    | <1             | 90                              |
| Water-washing                        | 5.0           | 0.2                    | 2              | 158                             |
| Distilled to 365° F.                 | 5.0           | 0.9                    | <1             | 166                             |

The lowering of the flash-point of the fuel by the volatile alcohol may be objectionable as an increased fire hazard. Therefore, it is desirable to remove the alcohol, except possibly in winter and in places where the fuel is normally stored in the presence of water. The sediment-forming tendency of the fuel is improved still further when the alcohol is removed by distillation.

#### EXAMPLE VII

Heating oil samples having properties as described in Example IV were treated with both isopropanol and an aqueous solution of sodium nitrite in 10% concentration. In one test the treatment with alcohol was followed by the treatment with nitrite and in the other test the order of treatments was reversed. The results of the tests were as follows:

| Treatment per Vol         | None  | 0.5 Vol. 10% NaNO <sub>2</sub> and 0.02 Vol. 1-C <sub>2</sub> H <sub>5</sub> OH | 0.02 Vol. 1-C <sub>2</sub> H <sub>5</sub> OH and 0.5 Vol. 10% NaNO <sub>2</sub> |
|---------------------------|-------|---------------------------------------------------------------------------------|---------------------------------------------------------------------------------|
| Sediment Tests:           |       |                                                                                 |                                                                                 |
| Initially Filterable      | 0.5   | 0.2                                                                             | 0.1                                                                             |
| Accel'd in Air            | 4     | <1                                                                              | <1                                                                              |
| Accel'd in oxygen         | 32    | 5                                                                               | 11                                                                              |
| Rusting Tendency, 12 Days | Heavy | None                                                                            | None                                                                            |

It is evident from the data that treatment with sodium nitrite followed by treatment with isopropanol is superior to treating with isopropanol alone as in Example V. It is also evident that treatment with isopropanol followed

by treatment with sodium nitrite for removal of the isopropanol is superior to the treatments shown in Example VI.

The present invention is thus broadly concerned with the treatment of liquid fuels with alcohols and with the removal of volatile or water-soluble alcohols from the treated fuels in order to improve the quality of the fuels, which are distillates like gasolines or heating oils. The alcohols, when not wanted in the treated fuels, can be removed by distillation or preferably by washing with an aqueous solution of a metal passivator. Preferred modifications of the present invention are to improve the stability of heating oils against formation of sediment by treating them with an alcohol and removing the alcohol with sodium nitrite. The treated fuels may be used without further treatment. They may be suitably blended with other fuels as desired. Suitable addition agents may be incorporated in the treated fuels for further improvement of quality. Such addition agents may be antioxidants. In gasoline fuels tetraethyl lead and lead scavenging agents can be used advantageously after the treatment according to the present invention. In diesel fuels, ignition promoters, for example alkyl nitrates, can be used after the treatments of this invention. In heating oils, suitable additives for use after the fuels have been treated in accordance with the present invention include sludge dispersers, detergents, antioxidants, pour-point depressors and rust-preventives. Examples of additives with rust-preventive properties are lecithin, oil-soluble petroleum sulfonates of sodium or calcium, and fatty acid esters of polyhydric alcohols, for example sorbitan mono-oleate. For instance, the addition of 0.9% isopropanol and 1.0% sorbitan mono-oleate to the heating oil described in Example IV decreased the accelerated sediment from 4 mgs. to 0.3 mg. per 100 ml. and completely prevented the rusting of iron for 12 days in contact with the treated oil.

What is claimed is:

1. The process for the production of an improved liquid hydrocarbon fuel oil of improved corrosion characteristics and increased stability comprising the steps of introducing a liquid hydrocarbon fuel containing at least 10% cracked gas oil and boiling in the range below about 700° F. into an initial treating zone, contacting said fuel in said zone with a treating agent consisting essentially of from about 0.5% to about 20% by volume of isopropanol based on the volume of said fuel while maintaining the temperature in said treating zone in the range of about 100° F. to about 180° F., passing the resulting mixture to a second treating zone, contacting said resulting mixture in said second treating zone with

an aqueous solution of a water-soluble metal-passivating alkali metal salt selected from the group consisting of nitrites, nitrates, chromates, bichromates, phosphates, phosphites, borates and benzoates to extract the isopropanol from said mixture, and separating improved hydrocarbon fuel from the resulting aqueous solution of water-soluble metal-passivating alkali metal salt and isopropanol.

2. The process according to claim 1 in which said metal-passivating alkali metal salt is sodium nitrite.

3. The process according to claim 1 in which the volume of said treating agent is from about 1% to about 5% based on the volume of said fuel, and in which said metal-passivating alkali metal salt is sodium nitrite.

4. The process for the production of an improved hydrocarbon fuel oil of improved corrosion characteristics and increased stability comprising the steps of introducing a liquid hydrocarbon fuel containing at least about 10% cracked gas oil and boiling in the range below about 700° F. into an initial treating zone, contacting said fuel with an aqueous solution of sodium nitrite, passing the resulting mixture to a second treating zone, contacting said mixture in said zone with a second treating agent consisting essentially of from about 1% to about 5% by volume of isopropanol based on the volume of said fuel while maintaining the temperature in said second treating zone in the range of about 100° F. to about 180° F., passing the resulting mixture to a third treating zone, contacting this resulting mixture in said third treating zone with a further portion of aqueous solution of sodium nitrite to extract the isopropanol from said mixture, and separating improved hydrocarbon fuel from the resulting aqueous solution of sodium nitrite and isopropanol.

#### References Cited in the file of this patent

#### UNITED STATES PATENTS

|           |               |               |
|-----------|---------------|---------------|
| 66,364    | Loomis et al. | July 2, 1867  |
| 685,895   | Wirth         | Nov. 5, 1901  |
| 1,256,537 | Dyer et al.   | Feb. 19, 1918 |
| 1,791,521 | Bjerggaard    | Feb. 10, 1931 |
| 1,822,351 | Krauch et al. | Sept. 8, 1931 |
| 1,899,042 | Malisoff      | Feb. 28, 1933 |
| 1,960,974 | Krauch et al. | May 29, 1934  |
| 1,968,842 | Malisoff      | Aug. 7, 1934  |
| 2,309,653 | Leum et al.   | Feb. 2, 1943  |

#### FOREIGN PATENTS

|         |               |              |
|---------|---------------|--------------|
| 169,573 | Great Britain | Oct. 6, 1921 |
|---------|---------------|--------------|